

G. RIGG.

REMOVING CADMIUM FROM ZINC ORE,  
APPLICATION FILED JULY 27, 1915.

1,161,886.

Patented Nov. 30, 1915.



Inventor:

Gilbert Rigg,  
by  
Jamie, Davis & Marin,  
Attorneys.

# UNITED STATES PATENT OFFICE.

GILBERT RIGG, OF PALMERTON, PENNSYLVANIA, ASSIGNOR TO THE NEW JERSEY ZINC COMPANY, OF NEW YORK, N. Y., A CORPORATION OF NEW JERSEY.

## REMOVING CADMIUM FROM ZINC ORE.

1,161,886.

Specification of Letters Patent. Patented Nov. 30, 1915.

Application filed July 27, 1915. Serial No. 42,210.

*To all whom it may concern:*

Be it known that I, GILBERT RIGG, a subject of the King of Great Britain, residing at Palmerton, Carbon county, State of Pennsylvania, have invented certain new and useful Improvements in Removing Cadmium from Zinc Ore; and I do hereby declare the following to be a full, clear, and exact description of the invention, such as will enable others skilled in the art to which it appertains to make and use the same.

The present invention relates to the removal of cadmium from zinc ore, for the purpose of recovering the cadmium and also for the purpose of obtaining a zinc ore product which is substantially devoid of cadmium and which can therefore be used in the manufacture of spelter in which cadmium is substantially absent.

20 In the accompanying drawing, I have shown, in general outline, a vertical section of apparatus utilizable for the practice of the invention.

In carrying out the invention, I preferably make use of a down-draft through the cadmium-containing roasted or naturally oxidized zinc ore treated. The bed of ore is located upon a suitable supporting grate surface, either of the stationary or traveling type, within a furnace structure wherein provision is made for effecting a down-draft through the charge.

In one form or modification of the invention, a layer of coal is placed on top of the layer of ore. This layer of coal is then ignited and a sufficient supply of air is drawn through the coal and the charge to bring the charge to the reacting temperature for cadmium reduction. The supply of air is then materially modified so that the reaction temperature referred to shall not be exceeded within the mass, except to the extent unavoidable at the surfaces of contact between the solid fuel and the zinc ore. Under these circumstances, the carbon monoxide generated reduces the cadmium oxid and the released cadmium is carried off with the issuing gases, in a vaporous condition, either as a metal or as an oxid, or (if sulfur is present) as a sulfid. It is received in any suitable condenser in which it may be recovered, in whole or in part, in combination with oxygen, sulfur, or other accompanying constituent capable of combining with it to form a stable deposit; as for instance, cad-

mium oxid or cadmium sulfid. Substantially all of the zinc which may be reduced at the surfaces of contact between the coal and the ore is caught and retained in the lower portion of the charge. The temperature of the lower portion of the charge, however, is sufficiently high to prevent the retaining of the cadmium therein, because of the lower volatilization point of cadmium.

In some instances, the layer of coal may be separated from the ore by a layer of inert material as, for instance, a layer of small pieces of burnt fire clay, or quartz. The main purpose of this interposed material is to prevent actual contact of the coal with the ore and, consequently, to prevent any reduction of zinc which might otherwise be incidental to the direct contact of the coal and ore.

Instead of superposing solid fuel upon the bed of zinc ore, igniting the fuel and drawing air downwardly through it and the ore, I may, in some instances, draw downwardly through the ore an ignited mixture of air with producer gas or other fuel gas until the ore reaches the temperature of reduction of cadmium but not of zinc. The air is then cut off and the reducing gas is alone drawn through the ore, thereby reducing and expelling the cadmium. The necessary temperature is maintained within the ore by periodically adding air to the gas and drawing the ignited mixture through the ore. The heating up of the ore to the necessary temperature, alternated with the passage of the reducing gas therethrough, may be proceeded with until the cadmium has been expelled.

In the case of ores containing sulfur, such as roasted blende ores, there is a tendency for the cadmium to combine with the sulfur and to form cadmium sulfid which is but slowly reducible by the gas. This can be compensated, in all of the instances hereinbefore referred to, by repeatedly alternating the conditions in the furnace from reducing to oxidizing, thus converting any cadmium sulfid formed during a reducing period to cadmium oxid during an oxidizing period. The cadmium oxid thus formed is then readily reduced and expelled during the next succeeding reducing period.

While I prefer, as hereinbefore indicated, to place the fuel layer upon the ore and to employ a down-draft, the fuel layer may in

some instances be placed below the ore layer and an updraft may be used. So also, the ignited mixture of producer gas and air, and the subsequent current of gas alone, may be passed upwardly instead of downwardly through the ore, although with lesser advantage.

It will be understood, of course, that the purpose of the invention is not only to 10 cover the cadmium, for the uses which cadmium has in the arts, but also to remove it as an impurity from the zinc ores containing it, so that it may not reappear in and deteriorate the spelter obtainable from the 15 zinc ores carrying it. The conditions of the practice permit both of these purposes to be effected without any substantial reduction and loss of zinc during the cadmium-expelling operation.

20. What I claim is:

1. The method of removing cadmium from roasted or naturally oxidized zinc ore, which comprises superposing, the one upon the other, a layer of fuel and a layer of cadmium-containing zinc ore, igniting the fuel and passing a body of air through the fuel and then through the ore until the ore is raised to the reduction temperature of cadmium but not of zinc, and continuing the 30 passage of air through the fuel and ore, for the removal of the cadmium, without substantial removal of the zinc; substantially as described.

2. The method of removing cadmium from roasted or naturally oxidized zinc ore, which comprises superposing, the one upon the other, a layer of fuel and a layer of cadmium-containing zinc ore, igniting the fuel and passing a body of air through the fuel 35 and then through the ore until the ore is raised to the reduction temperature of cadmium but not of zinc, and continuing the passage of air through the fuel and ore, for the removal of the cadmium, without 40 substantial removal of the zinc, the depth of the ore layer being made sufficient to catch and retain substantially all of the zinc which may have been reduced at the 45 surfaces of contact of the layers of fuel and ore; substantially as described.

3. The method of removing cadmium from roasted or naturally oxidized zinc ore, which comprises subjecting the ore to the reducing action of reducing gas passed 50 through the charge at a temperature sufficiently high throughout the charge to reduce and volatilize the cadmium and permit its expulsion from the charge, and sufficiently low at the exit zone for the reducing gas, to permit the charge to catch and retain any zinc that might otherwise be ex-

5 pelled with the cadmium; substantially as described.

4. The method of removing cadmium from roasted or naturally oxidized zinc ore, which comprises subjecting the ore to the reducing action of a down-draft of reducing gas passed through the charge at a temperature sufficiently high throughout the charge to reduce and volatilize the cadmium and 10 permit its expulsion from the charge, and sufficiently low at the exit zone for the reducing gas, to permit the charge to catch and retain any zinc that might otherwise be 15 expelled with the cadmium; substantially as described.

5. The method of removing cadmium from roasted or naturally oxidized zinc ore, which comprises subjecting the ore to the reducing action of a down-draft of reducing 20 gas passed through the charge at a temperature sufficiently high throughout the charge to reduce and volatilize the cadmium and permit its expulsion from the charge, and sufficiently low at the exit zone for the reducing gas, to permit the charge to catch and retain any zinc that might otherwise be 25 expelled with the cadmium, the reducing gas being produced by the ignition and combustion of a layer of fuel superposed upon the zinc ore charge; substantially as described.

6. The method of removing cadmium from roasted or naturally oxidized zinc ore, which comprises subjecting the ore to the reducing action of a down-draft of reducing 30 gas at a temperature sufficient to reduce and volatilize the cadmium without expelling any substantial quantity of the zinc, the reducing gas being produced by the ignition and combustion of a layer of fuel superposed upon the zinc ore charge with the interposition of a layer of inert material; substantially as described.

7. In the art of removing cadmium from roasted or naturally oxidized zinc ore by the reducing action of a reducing gas at a temperature sufficient to reduce and volatilize the cadmium without expelling any substantial quantity of the zinc, the method 10 of alternating reducing periods with oxidizing periods, so as to oxidize and render easily removable any cadmium sulfur compounds formed during the reducing periods; substantially as described.

In testimony whereof I affix my signature, in presence of two witnesses.

GILBERT RIGG

Witnesses:

JOHN C. PENNIE,  
M. A. BILL.